

## UNITED STATES PATENT OFFICE.

ERNEST G. JARVIS, OF PATERSON, NEW JERSEY, ASSIGNOR, BY MESNE ASSIGNMENTS,  
TO MERCO NORDSTROM VALVE COMPANY, OF SAN FRANCISCO, CALIFORNIA, A  
CORPORATION OF DELAWARE.

## ALLOY.

No Drawing.

Application filed April 13, 1923. Serial No. 631,889.

To all whom it may concern:

Be it known that I, ERNEST G. JARVIS, a citizen of New Jersey, residing at Paterson, in the county of Passaic and State of New Jersey, have invented certain new and useful Improvements in Alloys, of which the following is a specification.

The invention relates to an improvement in alloys.

10 One object of the invention is to produce a new and improved alloy characterized by its superior fitness for use in valves and other parts subjected to the effects of superheated and saturated steam and high temperatures generally, and to the effects of concentrated or dilute hot and cold acids. A further object of the invention is to produce an alloy characterized by having a high melting point, ability to withstand severe 20 shocks, great tensile strength and homogeneity of structure.

The alloy in its preferred composition consists of a mixture of the following metals in approximately the proportions specified, 25 namely:

|           | Per cent. |
|-----------|-----------|
| Tin       | 1         |
| Lead      | 2         |
| Iron      | 2         |
| 30 Copper | 60        |
| Nickel    | 25        |
| Zinc      | 10        |

Although I prefer to make the improved 35 alloy from the various metals in the proportions given above for the best results, not only as to the heat and acid resisting qualities of the alloy, its homogeneity of structure, its great tensile strength and ability to

withstand severe shocks, but also as to the adaptability of the alloy for casting, machining and the like operations, nevertheless I have found that an alloy satisfactory for the purposes of the invention may be made from these various metals within the following limits:—

|        | Per cent. |
|--------|-----------|
| Tin    | 1 to 3    |
| Lead   | 1 to 4    |
| Iron   | 2 to 6    |
| Copper | 60 to 65  |
| Nickel | 22 to 28  |
| Zinc   | 8 to 12   |

The metals composing the alloy are melted together and cast in the usual manner. The alloy may be employed for any purpose where the conditions require a non-corrosive, heat-resistant metal, which is impervious to superheated and saturated steam under high pressures and which is capable of withstanding without harm great stresses and severe and sudden shocks. Moreover, the alloy is easily machined.

I claim:

1. An alloy consisting of the following metals taken within the limits of approximately the proportions given: tin 1 to 3 per cent; lead 1 to 4 per cent; iron 2 to 6 per cent; copper 60 to 65 per cent; nickel 22 to 28 per cent; zinc 8 to 12 per cent.

2. An alloy consisting of a mixture of metals in approximately the following proportions: tin 1 per cent; lead 2 per cent; iron 2 per cent; copper 60 per cent; nickel 25 per cent; zinc 10 per cent.

ERNEST G. JARVIS.